

April 27, 1954

B. L. TRILICH

2,676,897

SELF-SEALING WRAPPING MATERIAL

Original Filed Nov. 7, 1949

2 Sheets-Sheet 1



Inventor  
Bertram L. Trilich  
By Fred G. Madlatty

April 27, 1954

B. L. TRILLICH

2,676,897

SELF-SEALING WRAPPING MATERIAL

Original Filed Nov. 7, 1949

2 Sheets-Sheet 2



Inventor  
Bertram L. Trillich  
By Fred Gersbach, Atty

## UNITED STATES PATENT OFFICE

2,676,897

## SELF-SEALING WRAPPING MATERIAL

Bertram L. Trillich, Winnetka, Ill., assignor to  
The Munising Paper Company, Chicago, Ill., a  
corporation of Ohio

Original application November 7, 1949, Serial No.  
125,973. Divided and this application June 20,  
1950, Serial No. 169,237

6 Claims. (Cl. 117—68)

1

This invention relates to a wrapping material especially adapted for wrapping small articles and more particularly to a quick-sealing, moisture-proof, wrapping paper for wrapping a comestible to maintain its moisture content. In its preferred aspects the invention relates to a quick-sealing, moisture-vapor-proof wrapping paper.

This application is a division of my copending application, Serial No. 125,973, filed November 7, 1949, now Patent No. 2,529,060.

The wrapping material of the present invention consists of a paper-thin flexible carrier sheet, preferably of paper, having a flexible coating of a moisture-proof material, preferably a moisture-vapor-proof material, on one side thereof and on the other side a flexible coating or film of a resinous self-adhering material which is substantially dry to the touch and substantially non-tacky but which is cohesive even under light pressure, and yet which is for all practical purposes non-adhesive to any surface such as paper, cellophane, wood, glass, metal, paint, rubber, etc., devoid of said material. The resinous self-adhering materials which may be used in accordance with the present invention are known materials and are usually termed "cohesive, substantially non-adhesive" materials. For convenience, these materials will be similarly referred to herein. Any of such resinous self-adhering materials may be used in accordance with the present invention.

The combination of a flexible water-proof coating on one side of a flexible carrier sheet and of a cohesive, substantially non-adhesive coating or film on the other provides a wrapping material for foodstuffs having desired moisture-proof or moisture-vapor-proof properties and a versatility and ease of use not heretofore present in any of the prior art wrapping materials, insofar as I am aware. The wrapping material of the present invention may be manipulated readily in sealing relationship about foodstuffs or dishes or other articles containing the same without the aid of heat or other extraneous expedients which entail skill and are inconvenient for the user.

In its preferred aspects the wrapping material of the present invention consists of a flexible, calendered paper sheet, one surface of which is coated with a flexible film or coating of a wax and the other with a film or coating of a resinous cohesive, substantially non-adhesive material such as a film or coating of a plasticized polyvinyl acetate composition disclosed in Patent No. 2,371,001, granted March 6, 1945.

Any paper-thin, flexible carrier sheet which lends itself for use in wrapping small articles may

2

be used in accordance with my invention, although paper is preferred as noted above. With such a sheet, the resinous cohesive, substantially non-adhesive material cooperates with the wax to seal any imperfections in the sheet and/or to impart the desired moisture-proof or moisture-vapor-proof properties to the sheet. When paper is used as the carrier sheet it is preferred that it be a lightly sized paper which permits some surface penetration of the resinous cohesive, substantially non-adhesive material. Other papers such as hard sized papers may, of course, be used. With such hard sized papers it may be necessary to overcome the effect of this sizing by the addition to the resinous material of a surface active agent to reduce the surface tension of the resin and to increase the wetting and penetrating power thereof. Any suitable surface active agent may be used for this purpose. Examples of suitable surface active agents are sodium lauryl sulphate, sodium cetyl sulphate, the sodium salt of the diethyl ester of sulfosuccinic acid (Aerosol OT), the sodium sulphate derivatives of 7-ethyl-2-methyl-undecanol-4 (Tergitol 4) and 3, 9 diethyl tridecanol-6 (Tergitol 7), decyl benzene sodium sulfonate (Santomerse 5), and phenyl-para-toluene sulfonate.

As pointed out above, any resinous cohesive, substantially non-adhesive material may be used in accordance with the present invention. Thus it may be a resinous cohesive material formed from co-polymers of polyvinyl acetate and polyvinyl chloride, polyvinyl acrylate, polyvinyl methacrylate, polyvinyl ethacrylate and like acrylates having from 1 to 5 carbon atoms in the alkyl group, polyvinyl ethers, polyvinyl ketones such as methyl vinyl ketone, polyvinyl alcohol, polyvinyl acetals such as formal, butyral, etc., and similar compounds containing a single ethylenic double bond,  $>C=C<$ , or a mixture of such compounds. The amount of cohesive material applied to the carrier sheet may be varied widely, say from about 0.2 lb. to 2 lbs. (solids) per 144 sq. yds. of carrier sheet.

The following is a further example of a cohesive, substantially non-adhesive material which may be used in accordance with the present invention.

Parts by weight

|                                                  |       |
|--------------------------------------------------|-------|
| Polyvinyl acrylate latex                         | 100.0 |
| Dibutanaphthyl p-phenylene diamine (antioxidant) | 1.0   |

Any suitable wax or wax-like material such as paraffin wax, beeswax, montan wax, carnauba wax, synthetic wax such as the high melting point

synthetic wax sold by Glyco Products Co., Inc., under the trade-mark Acrawax C, and the like may be used as the moisture-proof coating for the wrapping material of the present invention. This coating may be applied to the carrier sheet in any desirable manner, in aqueous emulsion form from solvent solution, or from molten bath, for example, as is well understood. Other suitable moisture-proof materials such as the known plastic compositions of wax and rubber may also be used, as may also the relatively high melting point microcrystalline waxes. When such waxes are combined with the cohesive, substantially non-adhesive materials on opposite sides of a paper carrier sheet, the sheet is rendered moisture-proof. As is known, microcrystalline waxes consist of amorphous, substantially saturated compounds that have been formed from high boiling point, non-saturated petroleum derivatives by way of polymerization and possibly by condensation (which products in the raw state are known commercially as petrolatum); and, more specifically, those higher melting point substances separated therefrom and sold as petroleum wax. These microcrystalline waxes may be used alone or they may be admixed with a material such as coumarone resin, phenol-formaldehyde resin, copal gum and the like, which will form a colloidal suspension or gel with the microcrystalline wax, to increase the inherent adhesiveness of the wax, as described in the Dreymann Patent No. 2,031,036.

The present invention will be fully understood from the foregoing and from the following description of a preferred illustrative embodiment of the invention and of some uses thereof, as illustrated in the accompanying drawings, wherein:

Figure 1 is a perspective view of a coated sheet of paper embodying the present invention;

Fig. 2 is an enlarged cross-sectional view thereof taken along the line 2-2 of Fig. 1;

Fig. 3 illustrates the use of the coated paper of Fig. 1 for wrapping a sandwich, the latter being shown as resting on the cohesive surface of the paper;

Fig. 4 is a cross-sectional view of the wrapped sandwich taken substantially along the line 4-4 of Fig. 3;

Fig. 5 is a similar cross-sectional view taken substantially along the line 5-5 of Fig. 4;

Fig. 6 illustrates the use of the paper of Fig. 1 for wrapping foodstuffs which are contained in an article such as a dish;

Fig. 7 depicts the package formed by wrapping the paper about the foodstuffs in the dish in accordance with the present invention; and

Figs. 8 and 9 illustrate modified embodiments of the coated sheets of the present invention.

In the drawings the numeral 10 designates a flexible paper sheet, preferably a lightly sized paper sheet which permits of some surface penetration, the numeral 11 designates a wax or other water-proof or moisture-vapor-proof coating, and the numeral 12 designates the cohesive, substantially nonadhesive coating, applied uniformly and lightly over the surface of the paper.

In the use of this coated paper to wrap comestibles, for example, a sandwich, the sandwich, indicated by the numeral 13, is placed upon the cohesive coating of the paper sheet adjacent one end and within the boundaries thereof, as illustrated in Fig. 3. The other end of the coated sheet is then folded over the sandwich so that

5 marginal portions of the cohesive coating of the folded sheet are in opposed relationship. A light pressure is then applied to the opposed surfaces of the cohesive coating by running the fingers lightly around the marginal portions of the folded paper, thereby completely sealing the sandwich within a moistureproof package, illustrated in Figs. 4 and 5.

10 In the use of the paper of the present invention to wrap foodstuff contained within a dish or other article, the article containing the foodstuff, indicated by the numeral 17, is placed upon the cohesive coating of the paper, as shown in Fig. 6, and the free ends of the paper are pulled up around the foodstuff and bunched together with the cohesive coating surfaces in opposing relationship, thereby enclosing the foodstuff in a water-proof package which may be placed in a refrigerator until ready for use.

15 Due to the moisture-proof or moisture-vapor-proof characteristics of the wrapping sheet of the present invention, foodstuffs wrapped within this sheet may be kept within a refrigerator for substantial periods of time, without desiccation or decay and without acquiring the flavors of other foodstuffs. The contents of the package may be readily removed either by cutting the wrapper or by pulling it apart at the joining surfaces. In the latter case, if care is exercised in pulling the 20 surfaces apart, the sheet may be re-used.

25 The coated paper sheet referred to above has the cohesive, substantially non-adhesive coating all over one surface thereof and the wax over the other surface and these sheets may be stacked 30 one upon the other without adherence, by placing the cohesive coating of one sheet in contact with the wax coating of another.

35 The versatility of the coated sheet to wrap various articles may be increased by applying additional zones of the cohesive, substantially non-adhesive coating on the side of the sheet containing the wax or other waterproof coating, as illustrated in Figs. 8 and 9. In making these sheets the paper or other carrier sheet is coated 40 on one side throughout the area thereof with a cohesive, substantially non-adhesive coating as before and a similar coating is applied to the margins or other desired portions of the opposite side. The wax is then applied to the carrier sheet 45 between the areas delineated by the zones of cohesive, substantially non-adhesive coating.

50 In Fig. 9, the cohesive, substantially non-adhesive coating 18 is applied all over the surface of one side of the carrier sheet and, additionally, 55 along the longitudinal margins 19 on the opposite sides. The wax coating 20 is applied to the carrier sheet over the area between the zones of cohesive, substantially non-adhesive coating. In the embodiment of the invention illustrated in Fig. 8, there are additional zones of cohesive, substantially non-adhesive coating 21 which extend 60 between the marginal zones 19 of cohesive, substantially non-adhesive coating, at intervals throughout the length of the sheet.

65 For convenience of the user any of the coated sheets described above may be vended in the form of a roll, illustrated in Fig. 8, and transverse perforations or score lines, illustrated by the score lines 22, may be provided to enable the user to tear a piece of this wrapping sheet from the roll. Where the wrapping sheet of the present invention is provided with cohesive, substantially non-adhesive coatings on both sides, as in Figs. 8 and 9, stacked individual sheets may be interleaved 70 with Holland cloth or other liner material, or the

coated wrapping sheet may be wound on the roll with a liner material (not shown) to prevent the opposed cohesive surfaces from adhering to one another, as is well understood.

I claim:

1. As a new article of manufacture, a moisture-proof sheet of self-sealing wrapping material adapted completely to encase an article and thereby seal the same against outside moisture, said article comprising a thin flexible paper sheet normally pervious to moisture, said sheet having on one surface thereof an exposed comparatively thin flexible wax film coating completely covering said surface and thereby imparting moisture-proof properties thereto and on its other surface an exposed flexible film of a cohesive, substantially non-adhesive resin, said last mentioned film covering the complete said other surface of the sheet and being substantially dry and non-tacky and yieldingly self-adhering when portions thereof are brought into engagement, but being non-adhesive to such surfaces as wood, glass and metal, the said non-tacky self-adhering film cooperating with said wax coating in moisture-proofing said paper sheet.

2. As a new article of manufacture, a moisture-proof sheet of self-sealing wrapping material adapted completely to encase an article and thereby seal the same against outside moisture, said article comprising a thin flexible carrier sheet, said sheet having on one surface thereof an exposed comparatively thin flexible wax film coating completely covering said surface and on its other surface an exposed flexible film of a cohesive, substantially non-adhesive resin, said last mentioned film covering the complete said other surface of the sheet and being substantially dry and non-tacky and yieldingly self-adhering when portions thereof are brought into engagement, but being non-adhesive to such surfaces as wood, glass and metal.

3. As a new article of manufacture, a moisture-proof sheet of self-sealing wrapping material adapted completely to encase an article and thereby seal the same against outside moisture, said article comprising a thin flexible carrier sheet, said sheet having on one surface thereof an exposed comparatively thin flexible micro-crystalline wax film coating completely covering said surface and on its other surface an exposed flexible film of a cohesive, substantially non-adhesive resin, said last mentioned film covering the complete said other surface of the sheet and being substantially dry and non-tacky and yieldingly self-adhering when portions thereof are brought into engagement, but being non-adhesive to such surfaces as wood, glass and metal.

4. As a new article of manufacture, a moisture-proof sheet of self-sealing wrapping mate-

rial adapted completely to encase an article and thereby seal the same against outside moisture, said article comprising a thin flexible carrier sheet, said sheet having on one surface thereof an exposed comparatively thin flexible wax film coating completely covering said surface and on its other surface an exposed flexible film of a cohesive, substantially non-adhesive material consisting essentially of a polyvinyl resin, said last mentioned film covering the complete said other surface of the sheet and being substantially dry and non-tacky and yieldingly self-adhering when portions thereof are brought into engagement, but being non-adhesive to such surfaces as wood, glass and metal.

5. As a new article of manufacture, a sheet of self-sealing wrapping material adapted completely to encase an article and thereby seal the same, said article comprising a paper-thin, flexible carrier sheet, said sheet having on one surface thereof an exposed comparatively thin flexible film of a non-adhesive fluid-impervious material of the class consisting of wax and wax-like materials completely covering said surface and on its other surface an exposed flexible film of a cohesive, substantially non-adhesive resin, said last mentioned film covering the complete said other surface of the sheet and being substantially dry and non-tacky and yieldingly self-adhering when portions thereof are brought into engagement, but being non-adhesive to such surfaces as wood, glass and metal.

6. As a new article of manufacture, a moisture-proof sheet of self-sealing wrapping material adapted completely to encase an article and thereby seal the same against outside moisture, said article comprising a thin flexible carrier sheet, said sheet having on one surface thereof an exposed comparatively thin flexible wax film coating completely covering said surface and on its other surface an exposed flexible film of a cohesive, substantially non-adhesive material consisting essentially of a plasticized polyvinyl acetate resin, said last mentioned film covering the complete said other surface of the sheet and being substantially dry and non-tacky and yieldingly self-adhering when portions thereof are brought into engagement, but being non-adhesive to such surfaces as wood, glass and metal.

References Cited in the file of this patent

UNITED STATES PATENTS

| Number    | Name                  | Date          |
|-----------|-----------------------|---------------|
| 2,027,436 | Kallander et al. .... | Jan. 14, 1936 |
| 2,337,939 | Sermattel ....        | Dec. 28, 1943 |
| 2,354,060 | Rhodes et al. ....    | July 18, 1944 |
| 2,364,875 | Schieman ....         | Dec. 12, 1944 |
| 2,439,481 | Martin ....           | Apr. 13, 1948 |
| 2,529,060 | Trillich ....         | Nov. 7, 1950  |